

Feb. 5, 1946.

H. J. ELMENDORF  
METHOD FOR IMPROVING THE DUCTILITY OF  
HIGH-CARBON-STEEL TEMPERED WIRE  
Filed Dec. 18, 1943

2,394,434

FIG. 2.



FIG. 1.



Inventor:  
HAROLD J. ELMENDORF,  
by John E. Jackson  
his Attorney.

## UNITED STATES PATENT OFFICE

2,394,434

METHOD FOR IMPROVING THE DUCTILITY  
OF HIGH-CARBON-STEEL TEMPERED  
WIREHarold J. Elmendorf, Cleveland, Ohio, assignor  
to The American Steel and Wire Company of  
New Jersey, a corporation of New Jersey

Application December 18, 1943, Serial No. 514,845

2 Claims. (Cl. 148—21.55)

This invention is for the purpose of increasing the ductility of high-carbon-steel tempered wire without materially changing its tensile strength and elastic limit.

It is to be understood that high-carbon-steel tempered wire is high-carbon-steel wire that has been continuously heat treated, the treatment consisting of austenitizing, quenching and tempering in straight line operation, the heat treating cycles being so chosen that the heat treated wire meets the desired specifications. The wire is usually thereafter coiled in bundles with a sufficient radius to keep the wire free from cold work strain due to its coiling. The wire is rendered substantially martensitic by suitably quenching the same and its structure is converted to substantially tempered martensite by any conventional tempering treatment, this providing the wire with the high tensile strength and elastic limit required of high-carbon-steel tempered wire. However, sometimes the wire does not have adequate ductility, and it is in such instances that the present invention comes into play.

According to the present invention, the high-carbon-steel tempered wire, free from cold work strain, is maintained at temperatures of from about 300° to 600° F. for a time controlled to increase its ductility without materially changing its tensile strength and elastic limit. The exact time of the treatment may be easily determined by tests although from about one to twelve hours is usually considered preferable. Furthermore, it will be found that for different compositions of high-carbon steel, different temperatures, within the range, provide the maximum increase in ductility, as contrasted to the thought that the maximum temperature will always provide the maximum ductility. The exact temperature best suited for a particular steel composition may also be easily determined by tests, it being deemed best that the wire be maintained within the defined range, at about the temperature predetermined by test as providing the maximum increase in ductility without materially changing the tensile strength and elastic limit for high-carbon-steel tempered wire of about the same chemical composition.

In the accompanying drawing:

Figure 1 graphically shows the effects produced by the invention on the proportional limit and ultimate tensile strength of five different compositions of high-carbon-steel tempered wire; and Figure 2 shows the effects on the ductility as indicated by the per cent reduction of area.

The various wires identified on the illustrated graphs involve the following compositions:

| Steel       | Per cent C | MN   | P     | S     | SI    | MO    | CR    | V     |
|-------------|------------|------|-------|-------|-------|-------|-------|-------|
| AISI-C 1066 | 0.64       | 1.04 | 0.029 | 0.022 | 0.205 | ----- | ----- | ----- |
| AISI-C 1065 | .64        | .75  | .012  | .033  | .13   | ----- | ----- | ----- |
| AISI-A 6145 | .45        | .85  | .010  | .021  | .25   | ----- | 1.03  | .17   |
| AISI-A 4068 | .66        | .60  | .013  | .025  | .19   | .25   | ----- | ----- |
| AISI-A 9280 | .60        | .76  | ----- | ----- | 2.00  | ----- | ----- | ----- |

In further explanation of the graphs, the points represented at 0° F. on both graphs are values obtained by testing the various specimens immediately after their tempering, and the various points represented at 90° F. in Figure 1 are values after the specimens had been held for 90 hours at room temperature, while the points at 80° F. in Figure 2 also represent values after the specimens were held for 90 hours at room temperature. Other than noted, the treatment time was in all instances one hour.

It will be seen that in all instances there is an increase in the ductility at temperatures between 300° and 600° F. without any material change in the elastic limit or tensile strength. Due to the time requirement the present invention is probably best carried out by batch heating methods in appropriate baking ovens with the wire in its usual coiled bundle form.

The present invention is to be distinguished from the practice of bluing coiled springs containing cold work strain resulting from the small-radius coiling required to produce the spring shapes. In this process the bluing is applied to steel containing cold work strain and results in raising the elastic limit of the metal. In the case of the present invention, what might be termed the "baking treatment" is not applied to the steel containing any material cold work strain at all and it does not affect the elastic limit materially.

I claim:

1. Maintaining high-carbon-steel tempered wire free from cold work strain at temperatures of from about 300° to 600° F. for a time controlled to increase its ductility without materially changing its tensile strength and elastic limit.

2. Maintaining high-carbon-steel tempered wire free from cold work strain at temperatures of from about 300° to 600° F. for a time controlled to increase its ductility without materially changing its tensile strength and elastic limit, the wire being maintained at about the temperature within said range predetermined by test as providing the maximum increase in ductility without materially changing the tensile strength and elastic limit for high-carbon-steel tempered wire of about the same chemical composition.

HAROLD J. ELMENDORF.